

Patented Sept. 18, 1928.

1,684,748

# UNITED STATES PATENT OFFICE.

HERBERT R. STRATFORD, OF CLEVELAND, OHIO, ASSIGNOR TO THE STRATMORE COMPANY, OF CLEVELAND, OHIO, A CORPORATION OF OHIO.

## SURFACING DISK.

No Drawing.

Application filed December 31, 1927. Serial No. 244,052.

The present invention, relating as indicated to surfacing disks, is particularly directed to a new and improved disk formed of a single material and intended for use in the surfacing, grinding and finishing of various panels and articles, such as sheet metal panels for use in automobile bodies, castings, machined articles and others. The principal object of the invention is the provision of a disk for the purposes referred to which shall be simple and inexpensive to manufacture, and which shall be formed of one or more layers of a single material. A further object of the invention is the provision of a disk which shall have an increased life and an improved bond between the surfacing material, such as abrasive, the elements which constitute the disk proper, such as the layer or layers of supporting material.

To the accomplishment of the foregoing and related ends, said invention, then, consists of the means hereinafter fully described and particularly pointed out in the claims; the following description setting forth in detail certain mechanism embodying the invention, such disclosed means constituting, however, but one of various mechanical forms in which the principle of the invention may be used.

Abrasive paper, such as sand paper, emery paper and the like, has long been used and consists of a layer of grains of a suitable abrasive secured, by means of an adhesive such as glue, varnish or the like, to a supporting backing formed of some light paper. In the use of such papers neither flexibility nor strength in any unusual degree was required or secured, but upon the introduction of machine grinding in which disks are mechanically driven to simulate or to improve upon the condition secured by grinding wheels, it is found necessary, in order to secure a suitable strength of material and a bond between abrasive and backing, to reinforce the paper disk with a layer of cloth which was usually interposed between the paper element and adhesive and abrasive. By means of this combination of materials a suitable flexibility in the disk was secured while still retaining a sufficient strength and resistance to buckling to permit such disks in some cases to be driven under very severe conditions from the center, while at the same time a strong bond was obtained between

the abrasive and the disk through the penetration of the adhesion in the cloth. This bond was sufficiently effective to prevent the early removal of the grains from the disk even at those portions of the disk in which repeated flexing was taking place.

Many millions of composite disks of the character described above have been made and used to a great advantage in grinding and finishing operations on all sorts of surfaces, the only objectionable feature of such disks being that they were expensive and difficult to manufacture. I have discovered that certain materials possessing certain characteristics may be employed without any reinforcing material and, contrary to the expectations and experience of experienced manufacturers of abrasive, my new disk is capable of holding its abrasion, even at those points where repeated flexing is going on, better and for a longer time than a composition disk consisting of bonded layers of the best paper stock, a suitable cloth and abrasive. Obviously, the elimination of one of the layers from the disk greatly simplifies the manufacture and lowers the cost, while at the same time an increased life and rubbing efficiency is secured, which in turn materially lowers the cost of the grinding operations to the user.

My improved disk consists, briefly stated, of a hydrated or hydrolyzed cellulose made by treating cellulose with a material capable of partially dissolving the cellulose, such for example as zinc chloride. In manufacturing this material old cotton rags are commonly employed as the raw material, these rags consisting of almost pure cellulose. These are pulped and formed into sheets in the ordinary manner and the sheets are then passed through a zinc chloride solution causing the partial solution of the fibres, and probably the outside of each individual fibre is partially dissolved, producing a gelatinous, and more or less adhesive, coating on each fibre. The sheets thus treated are then again passed through rolls to remove the excess zinc chloride solution and to compress the fibres tightly together. Subsequent treatment consists in removing the final traces of zinc chloride, which may be effected by washing the sheets with water, after which the sheets are hardened and dried. It will be understood that various other reagents may be employed instead of

the zinc chloride, provided that they also have a gelatinizing of parts of the fibres to produce a chemical and mechanical adhesion between the fibres during the treatment 5 which is far more effective in cementing the entire structure together than merely the ordinary mechanical adhesion secured through pressure in the ordinary paper stock. The result of this treatment of the 10 material is to greatly increase the strength, the density and the rigidity, and to lower the porosity while producing a structure which has little or no tendency to split or curl. This product is ordinarily referred 15 to as "hydrolyzed cellulose", or commercially as "vulcanized fibre".

I have found that a disk formed of a suitable layer of vulcanized fibre of certain characteristics when supplied with a coating 20 on one surface of grains bonded thereto by a suitable adhesion will dry perfectly flat and without any curling or splitting of the edges, is of almost precisely the desired 25 flexibility and rigidity and possesses a bond between abrasive and fibre which is sufficient to hold the abrasive in position even under the most severe service and for a length of time materially greater than the best composite disks of the paper stock and cloth 30 which are at present in common use, and which up to this time have been universally conceded to be the only type of disk capable of withstanding the extremely severe service to which these disks are put.

It will be understood that in certain cases this type of surfacing disk is secured at its center to a supporting pad or cushion formed of various materials, such as a layer of compressible material, such as felt, and a 40 support behind the felt, such as a plate of metal, and is then rotated at extremely high speed while the radially outer portion of the abrasive disk is pressed firmly against a surface to be treated, such for example as 45 a rough metal panel of pressed steel. This operation is an extremely severe one, since at its outer edge the disk is sometimes being rotated at a speed between 5000 and 10,000 ft. per minute over a surface of extremely 50 tough material which is being ground away by this operation while the power applied to the disk for effecting the rotation is applied at a point remote from the engagement between the disk and the work, namely, at 55 the center of the disk, a number of inches away from the point where the disk engages the panel. In addition to the torsional strains imposed on the disk between the center and the edge there is also an additional 60 strain imposed on the material when, as is frequently the case, the disk is running over a projecting weld or bend in the panel, which is thus causing the disk to flex back and forth at a speed some times in excess of 3600 flexures per minute. It is this flexing back

and forth in particular which causes the loosening and removal of the abrasive from the disk and the flexing is always present even when the disk is not operating against welds or irregular surfaces since the conditions of operation require a bending of that portion of the disk applied to the work which is resisted, but permitted to a certain extent, by the compressible supporting pad, against which the disk is used. It was because of this extremely severe service to which the disk is put that experienced abrasive manufacturers resorted to the expensive combination of a sheet of paper stock and a sheet of fabric to build up a composite disk which was expected to have, to a maximum degree, the particular characteristics of flexibility, torsional strength and ability to retain the bond between the abrasive grains and the cloth required in 80 such an article.

I have found that a very much superior disk can be formed from one or more layers of vulcanized fibre, depending upon the particular service to which the disk is to be put, 90 since a disk of this material has, in a high degree, the particular qualities or characteristics which various tests have indicated are the determining factors in the success of the composite disk, although these characteristics are either present to a greater degree in a disk of fibre alone, or certain other characteristics which detract from the life of a composite disk are missing from a disk 95 of fibre alone.

One desired characteristic which is apparently important and necessary in such a disk is that the disk be of dense material. Thus, the density should be such that the weight of the material per cubic centimeter 105 should be one gram or more. The tensile strength should average not less than 170 pounds longitudinally of the sheet of paper from which the disk is to be formed and 85 pounds transversely. Resistance to abrasion 110 is of considerable importance and tests show that the material employed should not lose more than 15 per cent by weight when abraded with an aloxite disk operated against a sheet of the material under a pressure of  $\frac{1}{16}$  of a pound for 100 revolutions. A further characteristic which I consider to be of considerable importance is the ability of the material to withstand rupture. My improved disk is capable of withstand- 115 ing rupture when a piece one foot square is clamped in a frame and a four-pound weight allowed to drop against the paper through a distance of four feet.

The improved life of my new disk formed 125 of the vulcanized fibre is also believed to be attributable in part to the absence of any capacity to stretch following the removal of the abrasive from the rotating edge of the disk and the pressing of this edge portion :

of the disk directly against the work. Close examination of partially used composite disks formed of paper stock and cloth indicate that after the abrasive grains have been 5 removed from the edge of the disk, allowing the layer of cloth to directly contact the work, this cloth is stretched and the stretching permits the strains to extend radially inward and also circumferentially to the adjacent 10 cent portions of the disk, loosening the abrasive disk earlier than it would otherwise be removed and producing a progressive destruction of the disk. In my present disk, the grains when removed from the paper 15 leave the paper, or rather the vulcanized fibre, which is then pressed against the work but which is not capable of being stretched as is the cloth, and hence does not transfer strains to the adjacent operating portions of 20 the disk. I believe that this difference between the composite and the unit disks accounts in a large part for the increased life of the present construction, and thereby presents the anomaly of a disk of supposedly 25 weaker and less rigid construction having a materially longer life than a disk of supposedly strong, tough and rigid construction.

The particular advantages of my improved disk may also be secured in a disk formed 30 of two adhesively joined sheets of relatively thin fibre, to the outer surface of one of which the abrasive is then bonded as before. Similarly, the same advantages may be secured either wholly or in part by adhesively 35 binding together a relatively thin layer of fibre and a layer of some other material, such, for example, as pattern board. In this

construction the abrasive grains are secured to the outer face of the fibre sheet as this possesses the surface qualities described 40 above, which assists in securing the long life required of such a disk, while the other sheet of different material acts as a reinforcing and may be built up in thickness to secure, in combination with the fibre sheet, the other 45 properties which have been found necessary in such disk.

Other modes of applying the principle of my invention may be employed instead of the one explained, change being made as regards 50 the mechanism herein disclosed, provided the means stated by any of the following claims or the equivalent of such stated means be employed.

I therefore particularly point out and distinctly claim as my invention:—

1. A surfacing element consisting of a sheet of hydrolyzed cellulose having a density of not less than one gram per cubic centimeter, and carrying a layer of grains 60 adhesively secured to one surface thereof.

2. A surfacing element consisting of a sheet of cellulose material provided with a layer of abrasive grains adhesively secured to one surface of said sheet, and the latter 65 having a tensile strength of not less than 170 pounds per square inch in one direction and of not less than 85 pounds per square inch in a direction at right angles to the 70 first.

Signed by me, this 29 day of December, 1927.

HERBERT R. STRATFORD.